# EUROPEAN PATENT SPECIFICATION

(11) **EP 4 389 969 B1**
(45) Date of publication and mention of the grant of the patent: **14.05.2025**
(21) Application number: 23209927.5
(22) Date of filing: 14.11.2023
(51) Int. Cl.: D21F 11/00, D21J 1/00, D21H 21/34, D21H 23/00, D21H 13/50, D21H 15/08

(54) **A METHOD OF PRODUCING A PLATE COMPOSITE WITH THE USE OF CELLULOSE AND CARBON PARTICLES WITH INCREASED FIRE RESISTANCE**
VERFAHREN ZUR HERSTELLUNG EINES PLATTENVERBUNDES UNTER VERWENDUNG VONZELLULOSE- UND KOHLENSTOFFPARTIKEL MIT ERHÖHTER FEUERBESTÄNDIGKEITEN
PROCÉDÉ DE PRODUCTION D'UNE PLAQUE COMPOSITE À L'AIDE DEPARTICULES DE CELLULOSE ET DE CARBONE À RÉSISTANCE AU FEU ACCRUE

(30) Priority: 28.11.2022 PL 44296422
(43) Date of publication of application: 26.06.2024
(73) Proprietor: Uniwersytet Przyrodniczy w Poznaniu, 60-637 Poznan (PL)
(72) Inventor: MAZELA, Bartlomiej, 61-058 Poznan (PL); GRZESKOWIAK, Wojciech, 62-023 Kamionki (PL); PERDOCH, Waldemar, 63-006 Sródka (PL)
(74) Representative: Augustyniak, Magdalena Anna

(56) References cited:
- CN-A- 107 523 078
- CN-A- 108 716 164
- US-A1- 2019 016 958

## Description

The present invention relates to a method of producing of a composite material made of cellulose and carbon particles, resulting in a plate composite with increased fire resistance.

The present invention may be used in the construction industry (as a cladding material), vehicular, water and air transportation (e.g., building up railroad compartments, furnishing tourist vehicles, boats, yachts, aircraft), as well as a specialized packaging material. Composite may be used specifically as a cladding material due to its unique properties (e.g. low density, small cross-sectional dimensions, barrier to fire, water, sound).

From the description of CN205950916 (U), a solution of layered elements is known, where a fire-resistant plywood was produced, in which the outer layers are made of fire-resistant impregnated wood veneers and the inner layer is made of fiberboard. In this solution, aluminum hydroxide was introduced into the inner layer in the form of granules. The layers were glued together using fire-retardant amine resin. According to the description, the layers can also be made up of paper made fire-resistant with melamine.

Utility model CN205369573 (U) discloses a fire-resistant board with a three-layer construction, including a resistant inner layer. The layers between each other are glued together by means of an glue. The outer layers may can be cladded on both sides. Another example is known from CN107523078A.

US 2019/0016958 A1 solution is known concerning the use of expanded graphite for the reduction of flammability, specifically for its use as a flame retardant agent, for materials and/or products consisting of, or comprising, wood fibers, fiber cellulose, wood powder, cellulose powder, wood granules, cellulose granules and/or polyolefin-based materials. Moreover, it relates to materials and/or products, consisting of, or comprising wood fibers, cellulose fibers, wood powder, cellulose powder, wood pellets, cellulose pellets and/or polyolefin-based materials. To reduce the flammability in materials and/or products, expanded graphite is embedded. The invention also relates to such an agent, specifically a fire retardant agent, wherein expanded graphite is used alone or in combination with a boric acid/borax/alkali salt mixture. Specifically favorable areas of application are binders, adhesives and/or materials, products and/or materials, products and/or intermediates containing in specifically polyolefin-based materials, preferably for damping (walls, floors, ceilings) and/or for fixing floors and walls.

A method of producing a plate composite with the use of cellulose and carbon particles with increased fire resistance is that
1. Particles rich in elemental carbon, i.e. with a carbon content >90%, selected from expanded graphite (EG) and carbon nanotubes (CNT), are dispersed in water in weight ratios ranging from 0.2:1 to 1:0.2. in an aqueous system. The weight ratio of carbon particles to water is from 1:1 to 100:1.
2. Cellulose pulp with a concentration of 1-25% in water is produced
3. A dispersed suspension of carbon particles is introduced into the cellulose pulp.
4. A composite is formed on a paper machine
5. The composite is dried and pressed

Wherein in the first step an aqueous dispersion of elemental carbon-rich particles (>90%) is produced, so that particles of expanded graphite (EG) and carbon nanotubes (CNT) are mixed, in weight ratios in the range of 0.2:1 to 1:0.2. in an aqueous system. The weight ratio of carbon particles to water ranges from 1:1 to 100:1, the EG/CNT dispersion is maintained in water for a period of 24 hours, and then the resulting particle dispersion is homogenized for 30-45 seconds using a homogenizer with a speed from 400 to 4000 rpm until a homogeneous water dispersion is obtained. The resulting homogeneous dispersion of particles is added to the simultaneously produced pulp in an amount of 1-75% by mass in relation to the total mass of the product and the mixture is further grounded for 10 s in the refiner.

The size of EG particles is in the range of 10 - 1000 micrometers, and the average length of CNT is 1.5 µm, and the diameter is 9.5 *10-9 m.

Wherein the pulp is produced in such a way that cellulose, in the form of sheets, is initially comminuted into particles size of 1-4 cm², soaked in deionized water for 24 hours, the weight ratio of cellulose to water is 1:10, and after 24 hours the cellulose is defibered in a defiberizer and water is added until the total cellulose to water ratio is at the level of 1:50
The homogeneous pulp is transferred to a sheet-forming apparatus and diluted with water to a mass concentration in the range of 2-20%, specifically 7.5%, and cellulose-carbon sheets are formed. Sheet forming is advantageously preceded by intensive mixing of the dispersion by the barbotage method, i.e., by passing air through the forming sieve from below at a pressure of 0.2-0.4 bar, and then the pulp is filtered out on a sieve with a mesh size of max. 0.25 cm. The formed sheets are then transferred to a dryer, where simultaneously excess water is sucked out and the sheet is pressed at a maximum temperature of 97°C in time up to 600 s at a pressure of max. -97kPa.

The resulting composite material based on cellulose fibers incrusted with carbon particles allows to achieve low cross-sectional dimensions and low density while maintaining high fire resistance qualities. These features are highly desirable for specialized applications.

The composite can be a single-layer material (photo 1.) or a multi-layer material, consisting of at least two layers, where at least one layer is the said composite material, and the layers are joined by any known binder or biobinder. The composite material can also constitute inner layers, outer layers or both at the same time. The composite material can also be combined with other layers made of other or the same materials, but characterized by different carbon to cellulose particle ratios (photo. 3).

The aim of the invention is, therefore, a composite in the form of a layer, as a finished product as such, or a system of layers made of cellulose incrusted with expanded graphite (EG) and carbon nanotubes (CNT), combined to form a plate-like composite material in which the cellulose fibers provide mechanical strength to the product and the carbon particles protect it from fire.

Table 1 shows examples of cellulose material variants with different carbon particle contents. **It was unexpectedly found that saturating the hydrophobic carbon particles with water, provided full homogeneity and uniform distribution in the cellulose mass, which in subsequent steps of the production of the composite material translated into the fire-resistant properties of the final product.**

### COMBUSTIBLE PROPERTIES OF THE COMPOSITE COMPONENT AND THE COMPOSITE AS THE FINAL MATERIAL

### Combustion properties of plate composite determined by the mini fire tube (MFT) method

The lowest value of mass loss (ML) and the exhaust gas temperature was shown by the cellulose-carbon layer formed in the system: cellulose:EG:CNT (M), with a maintained ratio of respectively: 1:1:1. The mass loss and exhaust gas temperature at the exit of the pipe were respectively: 5.3% and 115°C. In the other variants, the mass losses were higher (6-70%), as were the exhaust gas temperatures (96-315°C). Control samples comprising 5 and 10 g of cellulose showed the highest mass loss (about 99%). The exhaust gas temperature at the exit of the pipe reached a the highest value of about 400°C.

**It was unexpectedly found that the presence of both types of carbon particles (EG and CNT) in the cellulose layer translated into a synergistic effect in terms of fire protection.**

### Combustion properties of plate composite determined by the oxygen index (OI) method

Layer samples made of cellulose encrusted with EG and CNT tested by the oxygen index (OI) method showed high fire resistance. The maximum oxygen index value for the sample of cellulose encrusted with EG (at a cellulose to EG ratio of 1:2) was 75%. The lowest value (22.5%) was shown by a sample of cellulose encrusted with EG and EG/CNT in a 2:1 ratio. The control samples showed an OI value of 20%, making the latter qualify as combustible.

### Combustion properties of plate composite determined by mass loss calorimeter (MLC) method

Samples of cellulose encrusted with CNT (in a 2:1 ratio) tested by the MLC method achieved the highest HRR of about 126kW/m², while the control sample showed an HRR at the level of about 137kW/m². The cellulose sample encrusted with EG or EG/CNT (with a cellulose to carbon particle ratio of 1:2) showed the lowest HRR, regardless of the mass of the cellulose (5 or 10g). The values were as follows: 35 and 38 or 23 and 31 kW/m² for 5g cellulose, respectively: EG (1:2) and cellulose 10g: EG/CNT (1:2).

A 10g cellulose sample with CNT (cellulose to carbon particle ratio of 1:2) showed the longest time to ignition - 18 seconds. The cellulose sample encrusted with EG and CNT particles (5g cellulose: EG/CNT, 2:1) ignited the fastest, i.e. after about 3s.

Cellulose encrusted with carbon particles in a 1:1.5 or 1:2 ratio, where the carbon particles were an EG/CNT system in a 1:1 ratio, showed high fire resistance properties.

**The results confirmed the non-obviousness resulting from the MFT analysis, where a synergy effect was found in the case of cellulose encrusted with EG and CNT in the ratio of 1:0.75:0.75 and 1:1:1.**

### Combustion properties of layered composite determined by mass loss calorimeter (MLC) method

The three-layer composite, in which the core was a layer comprising different amounts of EG: the cellulose mass ratio to EG was 1:5 (8 BV), showed the best results, i.e., the maximum peak

HRR was 212 kW/m² at 290s, while the control variant (F) reached a value of 282 kW/m² at 260s.

The three-layer composite, in which the core constituted a layer of cellulose encrusted with EG/CNT in a 1:1:1 ratio to cellulose (10EG10CNT10C), characterized by the highest fire resistance among the materials tested. The maximum value of the heat release rate (HRR) was 154.07 kW/m², while the HRR peak of the composite containing only EG was 282 kW/m²

### Example 0

A method of producing a plate composite with the use of cellulose and carbon particles with increased fire resistance is that
1. Particles rich in elemental carbon (>90%) are dispersed in water, wherein the particles rich in elemental carbon being a mixture of expanding graphite (EG) and carbon nanotubes (CNT), in weight ratios in the range of 0.2:1 in an aqueous system. The weight ratio of carbon particles to water is from 1:1.
2. Cellulose pulp with a concentration of 1% in water is produced
3. A dispersed suspension of carbon particles is introduced into the cellulose pulp.
4. A composite is formed on a paper machine
5. The composite is dried and pressed

Wherein in the first step an aqueous dispersion of elemental carbon-rich particles (>90%) is produced, so that particles of expanded graphite (EG) and carbon nanotubes (CNT) are mixed, in weight ratios in the range of 0.2:1 in an aqueous system. The weight ratio of carbon particles to water is 1:1, the EG/CNT dispersion is maintained in water for a period of 24 hours, and then the resulting particle dispersion is homogenized for 30-45 seconds using a homogenizer with a speed from 400 to 4000 rpm until a homogeneous water dispersion is obtained. The resulting homogeneous dispersion of particles is added to the simultaneously produced cellulose pulp in an amount of 75% by weight in relation to the total mass of the product and the mixture is further grounded for 10 s in the refiner.

The size of EG particles is in the range of 10 - 1000 micrometers, and the average length of CNT is 1.5 µm, and the diameter is 9.5 *10-9 m.

Wherein the pulp is produced in such a way that cellulose, in the form of sheets, is initially comminuted into particles size of 1-4 cm², soaked in deionized water for 24 hours, the weight ratio of cellulose to water is 1:10, and after 24 hours the cellulose is defibered in a defiberizer and water is added until the total cellulose to water ratio is at the level of 1:50

The homogeneous pulp is transferred to a sheet forming apparatus and diluted with water to a mass concentration of 7.5%, and cellulose-carbon sheets are formed. Sheet forming is advantageously preceded by intensive mixing of the dispersion by the barbotage method, i.e., by passing air through the forming sieve from below at a pressure of 0.2-0.4 bar, and then the pulp is filtered out on a sieve with a mesh size of max. 0.25 cm. The formed sheets are then transferred to a dryer, where simultaneously excess water is sucked out and the sheet is pressed at a maximum temperature of 97°C in time up to 600 s at a pressure of max. -97kPa.

### Example 0'

A method of producing a plate composite with the use of cellulose and carbon particles with increased fire resistance is that
1. Particles rich in elemental carbon (>90%) are dispersed in water, wherein the particles rich in elemental carbon being a mixture of expanding graphite (EG) and carbon nanotubes (CNT), in weight ratios in the range of 1:0.2 in an aqueous system. The weight ratio of carbon particles to water is 100:1.
2. Cellulose pulp with a concentration of 25% in water is produced
3. A dispersed suspension of carbon particles is introduced into the cellulose pulp.
4. A composite is formed on a paper machine
5. The composite is dried and pressed

Wherein the first step an aqueous dispersion of elemental carbon-rich particles (>90%) is produced, so that particles of expanded graphite (EG) and carbon nanotubes (CNT) are mixed, in weight ratios in the range of 1:0.2 in an aqueous system. The weight ratio of carbon particles to water is 100:1, the EG/CNT dispersion is maintained in water for a period of 24 hours, and then the resulting particle dispersion is homogenized for 30-45 seconds using a homogenizer with a speed from 400 to 4000 rpm until a homogeneous water dispersion is obtained. The resulting homogeneous dispersion of particles is added to the simultaneously produced pulp in an amount of 1% by weight in relation to the total mass of the product and the mixture is ground for 10 s in the refiner.

The size of EG particles is in the range of 10 - 1000 micrometers, and the average length of CNT is 1.5 µm, and the diameter is 9.5 *10-9 m.

Wherein the cellulose pulp is produced in such a way that cellulose, in the form of sheets, is initially comminuted into particles size of 1-4 cm² size, soaked in deionized water for 24 hours, the weight ratio of cellulose to water is 1:10, and after 24 hours the cellulose is defibered in a defiberizer and water is added until the total cellulose to water ratio is at the level of 1:50

The homogeneous pulp is transferred to a sheet forming apparatus and diluted with water to a mass concentration in the range of 7.5%, and cellulose-carbon sheets are formed. Sheet forming is advantageously preceded by intensive mixing of the dispersion by the barbotage method, i.e., by passing air through the forming sieve from below at a pressure of 0.2-0.4 bar, and then the pulp is filtered out on a sieve with a mesh size of max. 0.25 cm. The formed sheets are then transferred to a dryer, where simultaneously excess water is sucked out and the sheet is pressed at a maximum temperature of 97°C in time up to 600 s at a pressure of max. -97kPa.

### EXEMPLARY EMBODIMENTS OF COMPOSITE LAYER (EXAMPLE 1-6) AND A COMPOSITE LAYER (EXAMPLE 7-19)

### Example 1

10 g of EG and 10 g of CNT were added to 10 g of comminuted and pre-milled cellulose. Obtaining the material was done as in examples 0 and 0'. The results obtained by the MFT method for mass loss were 5.32% in 60 s of measurement. The exhaust gas temperature for this variant was also comparable to the other examples, reaching 114.87⁰C in 60 s of measurement. Analysis of the results obtained by the LOI method indicates very high effectiveness of the material obtained. The oxygen index value was 58.97%, a nearly 3-fold increase compared to the control variant, which classifies the material as non-inflammable. Tests using MLC show that the average HRR peak was 22.81 kW/m², the time to ignition was 15.67s. For variants containing 10 g of cellulose and 20 g of EG and 10 g of cellulose and 20 g of CNT, the values of mass loss and exhaust gas temperatures measured by the MFT method were 6.35% (111,36°C) and 27.44% (211,32°C), respectively. Also, the HRR peak values in both cases were higher than for the variant containing 10 g of cellulose and 20 g of carbon additives (at a 1:1 ratio of EG to CNT). The values of these peaks were 38.06 kW/m² and 88.05 kW/m², respectively. These values demonstrate the positive interaction of the carbon additives used.

### Example 2

7.5 g of EG and 7.5 g of CNT were added to 10 g of comminuted and pre-milled cellulose. Obtaining the material was done as in examples 0 and 0'. Using the test method as in example one, high efficiency was achieved. The results obtained by the MFT method for mass loss were 6.84% in 60 s of measurement. The exhaust gas temperature for this variant was significantly lower compared to example 1, and was 98.99°C at 31 s of measurement. Analysis of the results obtained by the LOI method indicates very high effectiveness of the material obtained. The oxygen index value was 46.15%, classifying the material as non-inflammable. Tests using MLC show that the HRR peak value was 36.43 kW/m², the time to ignition was 9.33 seconds. For variants containing the same amount of cellulose and the same amount of single carbon additives, for the variant containing 15 g EG, the mass loss measured by the MLC method was 7.91% reaching a maximum exhaust gas temperature of 102.6°C. For the variant containing 15 g of CNT, the values were 29.26% and 202.09°C, respectively. The LOI values also classified these materials as non-inflammable. The HRR peak values for each additive were higher than for the variant containing 15 g of carbon additives (1:1 ratio) and amounted to 46.07 kW/m² for the variant of 10 g cellulose with 15 g EG and 94.52 kW/m² for the variant of 10 g cellulose and 15 g CNT.

### Example 3

A three-layer plywood containing a sheet of modified cellulose material with EG and cellulose in a 1:1 ratio as the inner layer was produced. The outer layers were face veneers made of Scots pine. Tests using MLC show the maximum HRR peak value was 214.40 kW/m² at 335 seconds, the time to ignition was 71 s. For the control test containing two layers of veneers without the middle layer and glued with the same resin, the HRR peak value was 330.96 kW /m2 at 210 seconds, time to ignition was 54 s.

### Example 4

A two-layer plywood was produced containing a sheet of modified cellulose material with EG, CNT and cellulose in a 1:1:1 ratio as one outer layer. The second outer layer was a venner of common pine wood. Tests using MLC show, the maximum HRR peak value was 41.27 280kW/m² at 280 seconds, the time to ignition was 207 seconds.

### Example 5

A three-layer plywood was produced containing a sheet of modified cellulose material with EG, CNT and cellulose in a 1:1:1 ratio as the inner layer. The outer layers were face veneers made of Scots pine. Tests using MLC show, the maximum HRR peak value was 154.07 kW/m² at 160 seconds, the time to ignition was 48 seconds. The control test was the same as in Example 7.

### Example 6

A three-layer plywood was produced containing a sheet of modified cellulose material with EG and cellulose in a 1:1 ratio as the inner layer. The outer layers were face veneers made of Scots pine. The sheet contained half as many components as example 7. Tests using MLC show, the maximum HRR peak value was 194.35 kW/m² at 265 seconds, the time to ignition was 51 s. The control sample was the same as in example 7.

### Example 7

A three-layer plywood was produced containing a sheet of modified cellulose material produced on an industrial scale (based on the description of composite layer manufacturing) with EG and cellulose in a ratio of about 1:5 as the inner layer. The outer layers were face veneers made of Scots pine. Tests using MLC show, the maximum HRR peak value was 241.88 kW/m² at 285 seconds, the time to ignition was 113 s. The control test was the same as in example 7.

### Example 8

A four-layer plywood was produced containing sheets of modified cellulose material produced on an industrial scale (based on the description of composite layer manufacturing) with EG and cellulose in a ratio of about 1:5 as the two inner layers. The outer layers were face veneers made of Scots pine. Tests using MLC show, the maximum HRR peak value was 231.19 kW/m² at 345 seconds, the time to ignition was 52 s. The control test was the same as in example 7.

### Example 9

A two-layer plywood was produced containing a sheet of modified cellulose material produced on an industrial scale (based on the description of composite layer manufacturing) with EG and cellulose in a ratio of about 1:5 as the outer layer. The second outer layer was a venner of common pine wood. Tests using MLC show, the maximum HRR peak value was 163.01 kW/m² at 190 seconds, the time to ignition was 51 s.

### Example 10

A three-layer plywood was produced containing a sheet of modified cellulose material produced on an industrial scale (based on the description of composite layer manufacturing) with EG and cellulose in a ratio of about 1:5 as the inner layer. The outer layers were face veneers made of Scots pine. Tests using MLC show, the maximum HRR peak value was 338.37 kW/m² at 255 seconds, the time to ignition was 83 s. For the control test containing two layers of veneers without a middle layer and glued with the same starch adhesive, the HRR peak value was 229.71 kW/m² at 295 seconds, the time to ignition was 82 s.

### Example 11

A three-layer plywood was produced containing a sheet of modified cellulose material produced on an industrial scale (based on the description of composite layer manufacturing) with EG and cellulose in a ratio of about 1:5 as the inner layer. The outer layers were face veneers made of Scots pine. Tests using MLC show, the maximum HRR peak value was 212.31 kW/m² at 290 seconds, the time to ignition was 81 s. The control test was the same as in example 17.

### Example 12

A three-layer plywood was produced containing a sheet of modified cellulose material produced on an industrial scale (based on the description of composite layer manufacturing) with EG and cellulose in a ratio of about 1:7.5 as the inner layer. The outer layers were face veneers made of Scots pine. Tests using MLC show, the maximum HRR peak value was 260.95 kW/m² at 360 seconds, the time to ignition was 70 s. The control test was the same as in example 17.

## Claims

1. A method of producing a plate composite with the use of cellulose and carbon particles with increased fire resistance **characterized in that**
1.1. particles rich in elemental carbon, i.e. with a carbon content >90%, selected from expanding graphite (EG) and carbon nanotubes (CNT), are dispersed in water in weight ratios ranging from 0.2:1 to 1:0.2. in an aqueous system, the weight ratio of carbon particles to water is from 1:1 to 100:1.
1.2. cellulose pulp with a concentration of 1-25% in water is produced
1.3. a dispersed suspension of carbon particles is introduced into the cellulose pulp.
1.4. a composite is formed on a paper machine
1.5. the composite is dried and pressed
wherein the EG/CNT dispersion is kept in water for a period of 24 hours, and further the resulting particle dispersion is homogenized for 30-45 s by means of a homogenizer with a rotation speed from 400 to 4000 rpm until a homogeneous water dispersion is obtained and the homogeneous particle dispersion is added to the cellulose pulp produced in parallel in an amount of 1-75% by weight based on the total mass of the product and the mixture is further grounded for 10 s in the refiner, and the cellulose pulp is produced in such a way that the cellulose in the form of sheets is initially comminuted into particles size 1-4 cm², soaked for 24 hours in deionized water, the weight ratio of cellulose to water is 1:10, and after 24 hours the cellulose is defibrated in a defiberizer and water is added until the total cellulose to water ratio is at the level of 1:50, then the homogeneous mass is transferred to a sheet forming apparatus and diluted with water to a mass concentration ranging from 2-20%, and cellulose-carbon sheets are formed.

2. A Method according to claim 1, **characterized in that** the EG particle size is in the range of 10 - 1000 micrometers,

3. A method according to claim 1, **characterized in that** the average length of the CNT is 1.5 µm and the diameter is 9.5 *10-9 m.

4. A Method according to claim 1, or 2 or 3, **characterized in that** the cellulose pulp is diluted with water in an amount of 7.5%,

5. A method according to claim 1, or 2, or 3, or 4, **characterized in that** the forming of the sheets is preceded by intensive mixing of the dispersion by the barbotage method, i.e., by passing air through the forming sieve from underneath at a pressure of 0.2-0.4 bar, and then the pulp is filtered out on a sieve with a mesh size of max. 0.25 mm, and then the formed sheets are then transferred to a dryer, where simultaneously excess water is sucked out and the sheet is pressed at a maximum temperature of 97°C in time up to 600 s at a pressure of max. -97kPa.

## Patentansprüche

1. Ein Verfahren zur Herstellung von Platten-Verbundwerkstoff unter Verwendung von Zellstoff- und Kohlenstoffpartikeln mit erhöhter Feuerbeständigkeit, **dadurch gekennzeichnet, dass**
1.1. die Partikel, die reich an elementarem Kohlenstoff sind, d. h. einen Kohlenstoffgehalt von >90 % aufweisen, aus expandierendem Graphit (EG) und Kohlenstoff-Nanoröhren (CNT) ausgewählt und in Wasser im Gewichtsverhältnis von 0,2:1 bis 1:0,2 in einem Wassersystem dispergiert werden, wobei das Gewichtsverhältnis von Kohlenstoffpartikeln zu Wasser 1:1 bis 100:1 beträgt,
1.2. Zellstoffbrei mit einer Konzentration von 1-25% in Wasser hergestellt wird,
1.3. eine dispergierte Suspension von Kohlenstoffpartikeln in den Zellstoffbrei eingebracht wird,
1.4. mittels einer Papiermaschine ein Verbundwerkstoff hergestellt wird,
1.5. der Verbundwerkstoff wird getrocknet und gepresst,
wobei die EG/CNT-Dispersion für einen Zeitraum von 24 Stunden in Wasser gelagert wird, und danach die so erzielte Partikeldispersion 30 bis 45 Sekunden mittels eines Homogenisators mit der Drehzahl von 400 bis 4000 U/min homogenisiert wird, bis eine homogene Wasserdispersion erzielt wird, und die homogene Partikeldispersion dem parallel hergestellten Zellstoffbrei in einer Menge von 1 bis 75 Gew.-%, bezogen auf die Gesamtmasse des Produktes, zugegeben wird und die Mischung weiter für 10 Sekunden in einem Refiner gemahlen wird, und der Zellstoffbrei in der Weise hergestellt wird, dass der Zellstoff in Form von Blättern zunächst in Teilchen der Größe 1-4 cm² zerkleinert wird, 24 Stunden lang in entionisiertem Wasser eingeweicht wird, wobei das Gewichtsverhältnis von Zellstoff zu Wasser 1:10 beträgt, und nach 24 Stunden wird der Zellstoff in einem Zerfaserer unter Zugabe von Wasser zerfasert, bis das Gesamtverhältnis von Zellstoff zu Wasser 1:50 beträgt, dann wird die homogene Masse in eine Vorrichtung zur Herstellung von Blättern überführt und mit Wasser auf eine Massenkonzentration von 2 bis 20% verdünnt, wodurch Blätter aus Zellstoff-Kohlenstoff gebildet werden.

2. Verfahren nach Anspruch 1, **dadurch gekennzeichnet, dass** die EG-Partikelgröße im Bereich von 10 bis 1000 Mikrometer liegt.

3. Verfahren nach Anspruch 1, **dadurch gekennzeichnet, dass** die durchschnittliche Länge der CNT-Partikel 1,5 µm und der Durchmesser 9,5 *10-9 m beträgt.

4. Verfahren nach Anspruch 1, 2 oder 3, **dadurch gekennzeichnet, dass** der Zellstoffbrei mit Wasser in einer Menge von 7,5 % verdünnt wird.

5. Verfahren nach Anspruch 1 oder 2 oder 3 oder 4, **dadurch gekennzeichnet, dass** der Formung der Blätter eine intensive Durchmischung der Dispersion im Barbotage-Verfahren vorausgeht, d. h. die Luft strömt von unter her durch das Sieb mit einem Druck von 0,2 - 0,4 bar, und der Brei so auf einem Sieb mit einer Maschenweite von max. 0,25 mm ausgefiltert wird, und dann werden die geformten Blätter in einen Trockner überführt, wo gleichzeitig überschüssiges Wasser abgesaugt und das Blatt bei einer Temperatur von maximal 97 °C innerhalb von maximal 600 s bei einem Druck von max. -97 kPa gepresst wird.

## Revendications

1. Procédé de fabrication d'une plaque composite à base de cellulose et de particules de carbone présentant une résistance accrue au feu, **caractérisé en ce que**
1.1. des particules riches en carbone élémentaire, c'est-à-dire dont la teneur en carbone est supérieure à 90%, choisies parmi le graphite expansible (EG) et les nanotubes de carbone (CNT), sont dispersées dans l'eau dans des rapports en poids allant de 0,2:1 à 1:0,2. dans un système aqueux, le rapport en poids entre les particules de carbone et l'eau est de 1:1 à 100:1.
1.2. production de pâte de cellulose avec une concentration de 1 à 25% dans l'eau
1.3. une suspension dispersée de particules de carbone est introduite dans la pâte de cellulose.
1.4. un composite est formé sur une machine à papier
1.5. le composite est séché et pressé
dans lequel la dispersion EG/CNT est maintenue dans l'eau pendant une période de 24 heures, et la dispersion de particules résultante est homogénéisée pendant 30-45 s au moyen d'un homogénéisateur avec une vitesse de rotation de 400 à 4 000 tr/min jusqu'à l'obtention d'une dispersion d'eau homogène et la dispersion de particules homogène est ajoutée à la pâte de cellulose produite en parallèle dans une quantité de 1-75% en poids sur la base de la masse totale du produit et le mélange est ensuite broyé pendant 10 s dans le raffineur, et la pâte de cellulose est produite de telle manière que la cellulose sous forme de feuilles est initialement broyée en particules de taille 1-4 cm², trempée pendant 24 heures dans de l'eau désionisée, le rapport pondéral entre la cellulose et l'eau étant de 10, et après 24 heures, la cellulose est défibrée dans un défibrateur et de l'eau est ajoutée jusqu'à ce que le rapport total cellulose/eau soit de 1:50, puis la masse homogène est transférée dans un appareil de formation de feuilles et diluée avec de l'eau jusqu'à une concentration massique de 2-20%, et des feuilles de cellulose-carbone sont formées.

2. Procédé selon la revendication 1, **caractérisé en ce que** la taille des particules EG est comprise entre 10 et 1 000 micromètres,

3. Procédé selon la revendication 1, **caractérisé en ce que** la longueur moyenne du NTC est de 1,5 µm et le diamètre de 9,5 *10-9 m.

4. Procédé selon la revendication 1, ou 2 ou 3, **caractérisé en ce que** la pâte de cellulose est diluée avec de l'eau dans une proportion de 7,5%,

5. Procédé selon la revendication 1, ou 2, ou 3, ou 4, **caractérisé en ce que** la formation des feuilles est précédée d'un mélange intensif de la dispersion par la méthode du barbotage, c'est-à-dire en faisant passer de l'air à travers le tamis de formation par le dessous à une pression de 0,2-0,4 bar, puis la pulpe est filtrée sur un tamis d'une taille de maille de max. 0,25 mm, puis les feuilles formées sont transférées dans un séchoir, où l'eau excédentaire est simultanément aspirée et la feuille est pressée à une température maximale de 97°C pendant une durée allant jusqu'à 600 s à une pression maximale de -97kPa.
